

## UNITED STATES PATENT OFFICE

2,380,253

## METHOD OF GRANULATING METALS

James P. A. McCoy, Milwaukee, Wis., assignor of  
one-half to Milwaukee Tool & Die Company,  
Milwaukee, Wis., a corporation of Wisconsin

No Drawing. Application February 22, 1943,  
Serial No. 476,773

1 Claim. (Cl. 83—91)

The present invention relates in general to improvements in the art of metallurgy, and relates more specifically to an improved method of heat treating metals to granulate the same.

The principal object of my present invention is to provide an improved process of readily and effectively reducing solid metals to granular condition.

It frequently becomes desirable in the art of metallurgy, to reduce certain solid metals and especially those having relatively low melting points, to more or less powdered or granular condition. While some metals may be granulated by impact or crushing, and others may be chemically reduced, while still others may be granulated by heating them to molten state and then depositing the same in cool liquid or the like, none of these and other prior methods are entirely satisfactory either because of the excessive power consumption and other costs involved, or because the final product cannot be uniformly reduced without production of excessive fines. Most of the previous metal granulating processes also involve considerable waste of the materials due to undesirable oxidation of the metals, and can only be exploited with the aid of relatively complicated and expensive equipment and materials. Some of the prior methods of granulating are also relatively slow and tedious by virtue of the fact that they involve batch treatment, thus introducing objectionable features into practically all of these previous processes of metal granulation.

It is therefore a more specific object of the present invention to provide a simple, inexpensive and efficient method of granulating solid metals in an expeditious manner and with minimum waste of materials.

Another specific object of my invention is to provide a new and useful process of heat treating metals to uniformly pulverize or granulate the same while avoiding excessive oxidation due to the heat treatment.

A further specific object of the invention is to provide an improved and simplified method of mechanically and continuously granulating certain metals, without involving chemical action or treatment.

Still another specific object of this invention is to provide an improved process of rapidly converting solid metals or the like, to uniform granular condition quickly, effectively and at minimum cost.

These and other specific objects and advantages of my present invention, will be clearly

apparent from the following detailed description of the procedure involved.

Although the invention may be restrictively described herein as being advantageously applicable in the treatment of certain metals with the aid of certain granulating agents, it is not my desire or intent to thereby unnecessarily limit the scope or utility of the improved method which may also be applicable for and with the treatment of other invention is, however, commercially applicable materials not specifically mentioned herein. The invention is, however, commercially applicable primarily in the treatment of metals and alloys having relatively low melting points, that is, below 1000° C.

In accordance with my present improved metal reducing or granulating method, the metal to be reduced may be either in the form of bars, ingots or a coating applied to other metal. This metal which is to be reduced is first heated so as to transform the same to a plastic condition, while being constantly agitated in the presence of a pulverulent wiping agent having mechanical affinity for the plasticized metal. This wiping agent should be continuously brought in contact with and caused to rub against the metal as it becomes plasticized, and will quickly convert the plastic metal to more or less granular form and will mechanically retain or hold the granules. The mixture of granular metal and wiping agent may then be removed from the heating zone after the agent has become mechanically saturated or laden with metallic particles or granules, whereupon the granular metal may be readily removed from the agent and the latter may be reutilized for subsequent granulation of other metal. In cases where the metal being treated, is apt to be undesirably affected by oxidation, the wiping agent may be mixed with other granular or fibrous carbonaceous substance or material so as to provide a reducing atmosphere of carbon-dioxide and an abundant bulk mixture capable of maintaining the metal constantly covered and concealed from excess oxygen such as might be contained in the ambient atmosphere.

While various types of wiping agent may be used in carrying on my improved process, I have found that when granulating metals such as tin or solder having relatively low melting points, pulverulent silica gel or flour, bentonite, carbon black, silicon carbide, various clays, or other materials, reduced to finely divided or pulverulent condition such as 100 mesh or finer, may be utilized. I have also discovered that the use of different wiping agents will result in variation in

the size of the metal granules, and the desired agitation and wiping action may be readily obtained in an externally heated rotary drum through which the mixed metal and wiping agent can be continuously advanced with a cascading action. The wiping agent may be circulated through the heating drum several times before being sufficiently laden with metal granules; and the granular or fibrous material which is added to the wiping agent for the purpose of preventing oxidation, may be sawdust or any other material which will carbonize and produce CO and CO<sub>2</sub> when subjected to the plasticizing temperature of the particular metal which is being treated, thus providing the desired reducing atmosphere. The final separation of the granular metal from the wiping mixture may be effected in any convenient manner, and when tin or solder is being reduced to granular condition, this final separation can be quickly effected by flotation in a bath of water wherein the tin or solder granules will settle by gravity while the wiping mixture may be floated off and reclaimed for further use. The foregoing procedure will permit rapid and continuous reduction of large quantities of metal to uniformly granulated condition with the aid of very simple equipment and at extremely moderate cost.

From the foregoing detailed description it should be apparent that my present invention provides an extremely simple and efficient method of granulating various metals without resorting to impact or crushing, and without excessive heating. Relatively inexpensive materials may be utilized in compounding the wiping mixture, and the metal may be reduced to either coarse or fine granular condition by selecting the proper

wiping agent, but in all cases the reduction is uniform and may be rapidly effected. Undesirable oxidation may also be eliminated by selecting proper carbonaceous materials for producing the desired reducing atmosphere while incidentally increasing the volume of the wiping mixture, and since the process is purely mechanical, the wiping ingredients can be quickly removed from the granulated or pulverized metal and reclaimed for further use. In order to produce best results and rapid action, the primary wiping agent should be fluffy and loose and incapable of packing, so that it will intimately contact all portions of the plasticized metallic surfaces. Actual exploitation of the improved method has demonstrated that tin and solder and other metals having relatively low melting points, can be quickly and effectively granulated in but a few minutes, and that a uniformly granular product results.

It should be understood that I do not desire to limit the present invention to the exact steps of the method or to the treatment of any particular material referred to and described herein for various modifications within the scope of the appended claims, may occur to persons skilled in the art.

I claim:

The method of producing granulated metal, which comprises, agitating the solid metals having melting points below 1000° C. while completely concealed in an abundance of saw dust and heating the mass to plasticize the metal, mixing silica gel with the concealed and plasticized metal to granulate the latter, and finally separating the granulated metal from the mixture.

JAMES P. A. McCOY.